

## UNITED STATES PATENT OFFICE.

ADOLF BECK AND KARL GERSBACH, OF BITTERFELD, AND OSKAR HERMANN WEBER, OF GRIESHEIM-ON-THE-MAIN, GERMANY, ASSIGNORS TO THE FIRM: CHEMISCHE FABRIK GRIESHEIM-ELEKTRON, OF FRANKFORT-ON-THE-MAIN, GERMANY.

## CASTING OXIDIZABLE METALS.

No Drawing.

Application filed May 25, 1922. Serial No. 563,717.

*To all whom it may concern:*

Be it known that we, ADOLF BECK and KARL GERSBACH, residing at Bitterfeld, and OSKAR HERMANN WEBER, residing at Griesheim-on-the-Main, Germany, citizens of Germany, have invented certain new and useful Improvements in Casting Oxidizable Metals, of which the following is a specification.

10 Our invention refers to the art of casting metals and more especially to means for preventing easily oxidizable metals such as magnesium and magnesium alloys from oxidizing in the mould.

15 The casting of easily oxidizable metals or metal alloys, as for instance of magnesium, involves the disadvantage that, more especially with sand moulds which strongly delay the effluence of heat from the molten metal, the metal surface remains for too long a period at a temperature which favours oxidation. In consequence of the slight shrinkage of the superficially solidified metal, an air gap may be formed between the metal and the sand mould which facilitates the admission of air from the atmosphere, whereby an ignition arising locally on the surface of the metal from any cause whatever can spread over the whole 30 surface of the metal. Thus worthless castings disfigured by burnt places are produced.

We have now ascertained the surprising fact, that by means of a suitable black wash brought onto the sand moulds and the cores thereof these undesirable oxidations can be completely obviated. As the result of extensive experiments we have found that such a black wash must in principle consist of materials which at the temperature of the cast metals give off gases or vapours more easily oxidizable than the metal and which either themselves or in their oxidized state do not affect the metal. In addition thereto these materials act particularly favourably by a special expenditure of heat being required for their evaporation or for the development of the gases owing to a process of decomposition, as hereby an accelerated chilling of the metal on the surface takes place.

*Example I.*—Magnesium oxalate, well dried and finely pulverised, is blown onto the dried sand mould or it is brought thereon after having been mixed with a non-aqueous, easily evaporating liquid. The cast metal effects the decomposition of this black wash into magnesia remaining on the layer of sand and into carbon monoxide with carbonic acid which when forming prevent the air from gaining access to the metal and which escape as carbonic acid.

*Example II.*—Pulverized sulfur is blown on to the dried sand mould or is deposited thereon in heated condition in such a manner that the sulfur will adhere to the sand mould in the form of minute drops, or else it may be sprayed on to the latter in suitable solution. The sulfur, upon coming into contact with the cast metal, evaporates and displaces and consumes the oxygen of the air by oxidizing to sulfur dioxide which escapes.

Castings produced in such a manner have a perfectly bright surface and are also free from porous spots underneath the skin.

The black wash according to the invention may be used in connection with all kinds of moulds.

We wish it to be understood that we do not desire to be limited to the particular substances and proportions described, for obvious modifications will occur to a person skilled in the art.

We claim:

1. The method of casting magnesium and alloys containing same, consisting in dusting the mould, prior to casting the metal, with a material capable of giving off, in contact with the molten metal, a gaseous substance, which is more easily oxidizable than magnesium.

2. The method of casting magnesium and alloys containing same, consisting in causing sulfur vapors to be developed in the mould in contact with the cast magnesium.

In testimony whereof we affix our signatures.

ADOLF BECK.  
KARL GERSBACH.  
OSKAR HERMANN WEBER.